

## UNITED STATES PATENT OFFICE

AUGUSTUS B. KINZEL, OF BEECHHURST, NEW YORK, ASSIGNOR TO ELECTRO METAL-LURGICAL COMPANY, A CORPORATION OF WEST VIRGINIA

## PROCESS OF CASE HARDENING

No Drawing.

Application filed May 26, 1930. Serial No. 455,955.

My invention relates to the production of nitrided layers on metals by heating the metals in nitrogen-containing agents, such as ammonia. It has particular reference to 5 an improved method of forming such hard wear-resistant cases.

The object of my invention is to provide means for accelerating and intensifying the action of nitriding gases on metal articles so 10 as to reduce the time required to produce a case of given hardness or thickness.

The case hardening of alloys is useful as a means of forming hard wearing surfaces on articles to be used for various machine 15 and tool parts. In order to avoid the formation of brittle cases or cause any other deleterious effect upon the material being treated the nitriding process is preferably carried out at low temperatures. To permit 20 the production of a satisfactory case at temperatures of the order of 460° C. to 580° C. it is often customary to alloy with the material to be treated small amounts of a promoting agent such as aluminum or vanadium. 25 A heating period of from 12 to 20 hours in a nitriding atmosphere such as ammonia is usually required to form a suitable case, the length of time of treatment increasing with a decrease in temperature. Such prolonged 30 heating which has been necessary to insure a proper reaction is expensive.

I have found that hard, nitrogen-containing cases may be produced in much less time by irradiating the nitriding gas and preferably also the surface of the specimen being treated with ultra-violet energy. Such energy may be generated by any of the common and convenient forms of electric arcs such as the carbon arc or the quartz mercury 40 vapor arc.

In the preferred form of my invention the specimen to be treated is placed in a chamber containing ammonia gas or other suitable nitriding agent. One side of the chamber may 45 be provided with a window of quartz glass or other material transparent to ultra-violet energy through which the nitriding atmosphere may be irradiated from a source outside the chamber. In this manner the specimen 50 may be so placed that its surface is ex-

posed to the energy transmitted through the window. In an arrangement where a continual passage of gas is maintained through the nitriding chamber suitable treatment may be effected by passing the nitriding gas 55 around an electric arc immediately prior to its entrance into the chamber.

With the use of ultra-violet energy as an accelerating agent I have been able to appreciably decrease the time required to effect 60 a suitable nitriding reaction. For example a hard nitride case may be formed on a specimen in four hours by means of my invention, whereas a similar specimen will show no hardening whatever when treated in the absence of ultra-violet energy for the same length of time. It is also possible to form a case in a given length of time, for instance 12 to 24 hours, with the use of ultra-violet radiation the depth of which is approximately 65 twice that formed under similar conditions without such radiation.

It is very probable that the nitriding gas, such as ammonia, is dissociated to a certain extent when exposed to ultra-violet radiation 75 forming a more active form of gas which causes the nitriding reaction to take place more readily. It also appears that the action of ultra-violet energy on the surface of the specimen being treated is a further contributing factor in accelerating the formation of a hardened case although I am unable to explain why this should be so. I have found for instance that when the nitriding atmosphere only is irradiated and the metal surface of the specimen is shielded from the direct radiation some improvement results, but when the specimen is also exposed the speed 80 of the nitriding reaction is much greater. 85

The invention should not be restricted by 90 the foregoing attempt to describe the theory involved. It will be evident that various modifications in the method as described may be made without departing from the spirit 95 of my invention as defined in the appended claims.

I claim:

1. The method of nitriding metal articles which comprises heating the articles in the presence of a nitriding agent and subjecting 100

said nitriding agent to ultra-violet radiation.

2. The method of nitriding metal articles which comprises heating the articles in the presence of a nitriding agent and irradiating 5 said articles while in said atmosphere with ultra-violet energy.

3. The method of nitriding metal articles which comprises subjecting the heated articles to an atmosphere of ammonia in a chamber, and irradiating said atmosphere with 10 ultra-violet energy from a source outside of said chamber.

4. The method of nitriding metal articles which comprises heating the articles in a 15 chamber containing an atmosphere of ammonia and subjecting said atmosphere and the surface of said articles to ultra-violet radiation through a portion of said chamber transparent to ultra-violet energy.

20 In testimony whereof, I affix my signature.  
AUGUSTUS B. KINZEL.

25

30

35

40

45

50

55